

(No Model.)

J. ENDRES & E. SCHOELLIG.

PROCESS OF MAKING ORNAMENTAL GLASS PANELS.

No. 409,834.

Patented Aug. 27, 1889.

fig. 1.



WITNESSES:

J. N. Rosenbaum.  
Carl Kay

INVENTORS  
Joseph Endres & Edward Schoellig  
BY  
George Preguer  
ATTORNEYS.

# UNITED STATES PATENT OFFICE.

JOSEF ENDRES AND EDUARD SCHOELLIG, OF LONG ISLAND CITY, NEW YORK.

## PROCESS OF MAKING ORNAMENTAL GLASS PANELS.

SPECIFICATION forming part of Letters Patent No. 409,834, dated August 27, 1889.

Application filed April 13, 1889. Serial No. 307,181. (No model.)

*To all whom it may concern:*

Be it known that we, JOSEF ENDRES and EDUARD SCHOELLIG, both of Long Island City, in the county of Kings and State of New York, 5 citizens of Germany, have invented certain new and useful Improvements in Processes of Making Ornamental Glass Panels, of which the following is a specification.

This invention relates to an improved process of making ornamental glass panels for furniture and for other purposes; and the invention consists of the following steps: first, coating the rear surface of two glass panels with oil or other paint; secondly, placing said 15 painted surfaces in contact with each other while moist and removing the same so that the uncolored figures form on the same; thirdly, coating said uncolored figures with a paint of different color; fourthly, varnishing the 20 whole back surface.

In the accompanying drawings, Figure 1 represents a vertical transverse section of two glass panels shown as painted on the back and placed in contact with each other. Fig. 25 2 represents rear elevations of said panels after they are separated from each other, Figs. 1 and 2 representing the second and third stages or process; and Fig. 3 is a vertical transverse section of the glass panels 30 shown as finished and provided with a suitable backing of wood.

Similar letters of reference indicate corresponding parts.

In carrying out our improved process of ornamenting glass panels A, which are intended to be used as a substitute for wood in furniture and for similar applications, glass plates of the required size are first properly cleaned and then painted on the back with oil or other 35 40 paint B, corresponding to the color of any desired wood. The so-painted surfaces are placed while in moist condition back to back and then removed quickly, so that the arbit-

rary figures C are formed on the surface of each plate, which figures contain no color, the 45 color being crowded by the suction exerted on the same in separating the plates in thicker layers onto the remaining surface of the plates. Another colored paint, different from the one first applied, is then given to 50 the rear surface of the plates, this color representing the grain of the wood. The entire rear surface of the panel is then coated with a suitable protecting varnish and the same, either backed with wood or other plates D, 55 inserted directly into their proper places in the furniture or other articles in which they are to be used. Glass panels ornamented in this manner present a very ornamental appearance and are very durable, as they do 60 not shrink or change, while they can be readily cleaned and require no polishing, like the surface of wood.

Having thus described our invention, we claim as new and desire to secure by Letters 65 Patent—

The process herein described of ornamenting glass panels, which consists of the following steps: first, coating the rear surfaces of two glass plates of equal size with oil or other 70 75 color; secondly, placing the painted surfaces in contact and separating the same, so as to produce uncolored figures of irregular size on both plates; thirdly, painting the uncolored portions with a color different from the first applied, and, lastly, covering the entire rear surface of the panels with a protecting coating of varnish, substantially as set forth.

In testimony that we claim the foregoing as our invention we have signed our names in 80 presence of two subscribing witnesses.

JOSEF ENDRES.  
EDUARD SCHOELLIG.

Witnesses:

PAUL GOEPEL,  
JOHN A. STRALEY.